

1

3,364,270

**STABILIZATION OF METHYL CHLOROFORM**  
 Milton J. Blankenship, Midland, and Ralph McCarthy,  
 Bay City, Mich., assignors to The Dow Chemical Company,  
 Midland, Mich., a corporation of Delaware  
 No Drawing. Filed Oct. 27, 1965, Ser. No. 505,419  
 4 Claims. (Cl. 260—652.5)

**ABSTRACT OF THE DISCLOSURE**

Methyl chloroform is stabilized in the presence of aluminum by incorporating in the solvent an inhibiting amount of a cyanobenzaldehyde.

This invention relates to the stabilization of methyl chloroform. More particularly, the present invention relates to the stabilization of methyl chloroform in the presence of aluminum.

It is known that methyl chloroform reacts violently with aluminum to form tars and gaseous reaction products.

It has now been found that this reaction may be substantially retarded or prevented by incorporating an inhibiting amount of a cyano-benzaldehyde compound into the methyl chloroform. Ortho-, para- and meta-cyano-benzaldehyde may each be used alone or in any combination. Only an amount of cyano-benzaldehyde compound sufficient to retard or stop the reaction of aluminum and methyl chloroform is required. Ordinarily, amounts of from about 0.5 to 10-15 percent by weight (based on the total weight of the composition) of cyano-benzaldehyde compound may be incorporated into the methyl chloroform. The preferred concentration of cyano-benzaldehyde compound in the methyl chloroform is from about 1.0 to 5.0 percent by weight (based on the total weight of the composition).

The cyano-benzaldehyde inhibitor compounds of the invention may be used alone or in combination with other non-reactive conventional inhibitors. Such cyano-benzaldehyde compounds are superior inhibitors when compared with related aldehydes, such as benzaldehyde.

The following examples are submitted for the purpose of illustration only and are not to be construed as limiting the scope of the invention in any way.

*Examples I and II*

Different amounts of cyano-benzaldehyde compounds were added to 10 milliliter samples of 1,1,1-trichloroethane. Concentrations were calculated as weight percents. An aluminum coupon [designated alloy 1100,<sup>1</sup> 18 gage

2

(approximately 0.04 to 0.05 inch thick by 2½ inches by ½ inch)] was immersed in each test solution and scratched with a sharp tool beneath the surface of the test liquid. The coupon was observed visually and the results recorded in Table 1 according to the following standards:

| Key number: | Indicated result                                           |
|-------------|------------------------------------------------------------|
| 3           | No reaction.                                               |
| 2           | Reaction starts but subsides (or stops) within 10 minutes. |
| 1           | Reaction slows down but continues after 10 minutes.        |
| 0           | Little or no inhibition; violent reaction.                 |

15

TABLE 1

| Ex. No. | Compound                                                         | Concen-<br>tration<br>(Weight<br>percent) | Result |
|---------|------------------------------------------------------------------|-------------------------------------------|--------|
| I.....  | Ortho-cyano-benzaldehyde (C <sub>7</sub> H <sub>5</sub> NO)..... | 3.65                                      | 3      |
|         |                                                                  | 2.74                                      | 3      |
|         |                                                                  | 1.82                                      | 3      |
|         |                                                                  | 1.59                                      | 2      |
| II..... | Para-cyano-benzaldehyde.....                                     | 3.65                                      | 3      |
|         |                                                                  | 2.74                                      | 3      |
|         |                                                                  | 1.82                                      | 3      |
|         |                                                                  | 1.36                                      | 3      |
|         |                                                                  | 1.12                                      | 3      |

30

We claim as our invention:

1. A composition inhibited against attack by aluminum which comprises methyl chloroform and an inhibiting amount of a cyano-benzaldehyde.
2. An inhibited composition according to claim 1 which contains 0.5 to 15 percent by weight of ortho-cyano-benzaldehyde.
3. An inhibited composition according to claim 1 which contains 0.5 to 15 percent by weight of para-cyano-benzaldehyde.
4. An inhibited composition according to claim 1 which contains 0.5 to 15 percent by weight of meta-cyano-benzaldehyde.

**References Cited**

**UNITED STATES PATENTS**

- 2,997,507 8/1961 Monroe et al. ----- 260—652.5  
 50 3,128,315 4/1964 Hardies ----- 260—652.5

**OTHER REFERENCES**

Every et al.: "Materials Protection," vol. 3 (9), pp. 46 and 47 (1964).

55 LEON ZITVER, Primary Examiner.

M. JACOB, Assistant Examiner.

<sup>1</sup> Aluminum alloy 1100 (standard designation of the Aluminum Association) is composed of (percent by weight):

1. 99.00 percent Aluminum (minimum)  
 2. 1.0 percent Si and Fe (maximum)  
 3. 0.20 percent Cu (maximum)  
 4. 0.05 percent Mn (maximum)  
 5. 0.10 percent Zn (maximum) } Total: less than 1.0 percent.